

Patented Jan. 18, 1927.

1,614,618

# UNITED STATES PATENT OFFICE.

HENRY JOSEPH, OF PITTSBURGH, PENNSYLVANIA, ASSIGNOR TO UNITED STATES SAND PAPER COMPANY, OF WILLIAMSPORT, PENNSYLVANIA, A CORPORATION OF PENNSYLVANIA.

## SHEET ABRASIVE MATERIAL.

No Drawing.

Application filed June 26, 1926. Serial No. 118,860.

This invention relates to improvements in sheet abrasive material such as sandpaper, emery cloth, etc.

The new sheet abrasive material is of a composite character and contains an inflammable or combustible binder for binding the abrasive to the flexible backing, but the composite sheet abrasive is nevertheless as a whole fire proof or fire resistant.

10 The new sheet abrasive material has the flexible backing, such as paper or cloth, treated so as to make it fire proof or fire resistant, and the abrasive itself is also fire proof or fire resistant, so that the combustible 15 or inflammable cementing material which secures the abrasive to the flexible backing, is protected on one side by the abrasive and on the other side by the fire proof backing. The cementing material, although inflammable or combustible, is nevertheless thereby 20 so protected that the composite sheet abrasive as a whole may be considered to be fire proof or fire resistant. When sheets of the abrasive are stacked together, the fire proof 25 abrasive comes in contact with the fire proof or fire resistant backing; and, during use of the abrasive, the combustible adhesive, or cementing material, is likewise protected on both sides by incombustible or fire proofed 30 material.

The cementing material employed may be a material such as glue, either alone or combined with other substances, or it may be a cementing material which is water resistant or water repellent, such as an adhesive containing resin, oils, etc. Such cementing material, both water soluble and water insoluble, are known in the art.

35 The cloth or paper or other backing may be fire proofed in various ways. For example, fire proofing materials may be compounded with or used to impregnate the backing, and these materials may be either organic or inorganic compounds of suitable 40 character to render the backing substantially fire proof. For example, the fire proofing materials may be inorganic salts, such as for example, ammonium phosphate or ammonium sulfate, or organic compounds such as 45 for example, triphenyl phosphate.

The treatment of the paper or cloth or other backing with the fire proofing material may be effected in various ways. For example, the cloth or paper backing may be

treated or impregnated with a solution of 55 the fire proofing agent or agents, or the fire proofing agent or agents may be used and incorporated into the paper or cloth during its manufacture in order to render it fire proof or fire resistant. A saturated aqueous 60 solution of ammonium sulfate is satisfactory for this purpose. The solution may be applied hot or cold to the paper or fabric, and the treated paper or fabric then allowed to dry in the air, or dried in a drying room, 65 so that the backing is in a dry state before the binder or adhesive is applied.

70 While the fabric or paper backing may be fire proofed only on the back side and may be left unfireproofed on the side to which the adhesive is applied, it may nevertheless advantageously be treated as a whole so that both sides of the paper or fabric backing are fire proofed before the adhesive or cementing material is applied thereto.

75 After the paper or fabric backing is rendered fire proof, the cementing or adhesive material may be applied thereto, and the abrasive, such as emery powder, glass powder, etc., may then be applied and the resulting product dried or cured in the usual manner.

80 In order that the composite product of the invention may be water proof as well as fire proofed, the paper or cloth or other backing 85 may be subjected to a water proofing treatment as well as to a fire proofing treatment. For example, the cloth or paper backing may be treated with a solution of a suitable varnish or other water proofing compounds, 90 and the treatment of the fabric or paper with the fire proofing agent may be carried out simultaneously, or the two operations may be carried out successively. In either case, the backing will be both water proofed 95 and fire proofed; and, where the adhesive or cementing material is also of a water proof character, such as resin and oil composition, the product as a whole will be water proof. In such case, the composite 100 product will be both water proof and fire proofed, although containing a cementing material which is not itself fire proofed, but which is nevertheless effectively fire proofed by enclosing it between the fire proof abrasive and the fire proof or fire resistant backing.

105 In my U. S. Patent No. 1,591,001, dated

June 29, 1926, I have described and claimed a flexible sheet abrasive material in which the adhesive is itself fire proofed. The present invention is differentiated from that set forth in my said patent by the fact that the adhesive material is not itself compounded with fire proofing material or otherwise directly fire proof; but it is nevertheless so confined between the fire proof abrasive and the fire proofed backing that it is effectively fire proof.

I claim:

1. A flexible sheet abrasive material comprising a flexible backing which is fire proof or fire resistant, an abrasive which is also fire proof or fire resistant, and a combusti-

ble adhesive uniting the abrasive to the backing.

2. A flexible sheet abrasive material comprising a flexible fire proofed or fire resistant 20 backing, an abrasive which is also fire proof or fire resistant and a combustible water proof adhesive for securing the abrasive to the backing, and the backing also being water proofed, whereby the composite product as a whole is water proof, and whereby the combustible adhesive is confined between fire proof or fire resistant layers of material. 25

In testimony whereof I affix my signature.

HENRY JOSEPH.